# EUROPEAN PATENT SPECIFICATION

(11) **EP 2 408 951 B1**
(45) Date of publication and mention of the grant of the patent: **03.05.2017**
(21) Application number: 10716121.8
(22) Date of filing: 17.03.2010
(51) Int. Cl.: C25C 5/02

(54) **METHOD FOR OBTAINING COPPER POWDERS AND NANOPOWDERS FROM INDUSTRIAL ELECTROLYTES INCLUDING WASTE INDUSTRIAL ELECTROLYTES**
VERFAHREN ZUM ERHALT VON KUPFERPULVERN UND -NANOPULVERN AUS TECHNISCHEN ELEKTROLYTEN EINSCHLIESSLICH ABFÄLLEN TECHNISCHER ELEKTROLYTE
PROCÉDÉ POUR OBTENIR DES POUDRES ET DES NANOPOUDRES DE CUIVRE PROVENANT D'ÉLECTROLYTES INDUSTRIELS, Y COMPRIS DES ÉLECTROLYTES INDUSTRIELS USÉS

(30) Priority: 20.03.2009 PL 38756509
(43) Date of publication of application: 25.01.2012
(73) Proprietor: Nano-Tech SP. Z O.O., 64-100 Leszno (PL)
(72) Inventor: LOS, Przemyslaw, PL-55-040 Zurawice (PL); LUKOMSKA, Anela, PL-01-466 Warszawa (PL); PLEWKA, Anna, PL-03-990 Warszawa (PL)
(74) Representative: Gill Jennings & Every LLP
(86) International application number: PCT/PL2010/000022
(87) International publication number: WO 2010/107328

(56) References cited:
- CN-A- 1 686 645
- YU ET AL: "Electro-reduction of cuprous chloride powder to copper nanoparticles in an ionic liquid" ELECTROCHEMISTRY COMMUNICATION, ELSEVIER, AMSTERDAM, NL LNKD- DOI:10.1016/J.ELECOM.2007.01.050, vol. 9, no. 6, 1 June 2007 (2007-06-01), pages 1374-1381, XP022089829 ISSN: 1388-2481
- O. GLADYSZ: "The electrochemical nucleation of copper on disc-shaped ultramicroelectrode in industrial electrolyte" ELECTROCHIMICA ACTA, vol. 54, 2 July 2008 (2008-07-02), pages 801-807, XP002585180
- LUKOMSKA A ET AL: "Shape and size controlled fabrication of copper nanopowders from industrial electrolytes by pulse electrodeposition" JOURNAL OF ELECTROANALYTICAL CHEMISTRY AND INTERFACIALELECTRO CHEMISTRY, ELSEVIER, AMSTERDAM, NL LNKD- DOI:10.1016/J.JELECHEM.2009.09.029, vol. 637, no. 1-2, 15 December 2009 (2009-12-15), pages 50-54, XP026771924 ISSN: 0022-0728 [retrieved on 2009-10-02]

## Description

The object of the invention is the method for obtaining copper powders from industrial electrolytes, including electrolytes which are the waste products of electroplating process, chemical, mining and smelting industry. Waste waters from the copper electrorefining and electroplating processes can be used in a very wide range.

Nanopowders are products of a very high value and their production and application is an important and developing field.

Copper powders and nanopowders are used as additions to polymers, lubricants, dye, antibacterial agents and microprocessor connections. Nanopowders of copper or its alloys can be used in microelectronics and as sorbents in the radioactive waste purification as well as a catalyst in fuel cells.

Nanopowders can be metal particles, metal oxide or organic complex smaller than a micrometer (at least one linear dimension). Production of nanopowders of a well-defined structure and controlled particles size is significant because of requirements that are to be fulfilled by the materials used in different fields of material engineering.

One of the currently used methods for obtaining copper nanopowders is electrochemical reduction method (electrodeposition). Electrolytic manufacturing of nano-siructured foil and deposits is presented in other patents.

For example in the patent CN 17107372005 copper foil made of copper nano-crystals of a size of about 150 nm has been obtained in the process of direct-current electrolysis in the following conditions: metal cathode, temperature 25-65°C, electrolyte flow rate 0.5-5.0 m/s, cathodic current density 0.5-5.0 A/cm². The electrolyte has been composed of the following additions: 1-15 mg/l thiourea, 1-15mg/l animal glue, 0.1-5.0 mg/l chloride ions and others.

The electrolytic method has been presented in the patent US 2006/0021878. The presented method for obtaining copper of great hardness and good electrical conductivity consists in pulse electrolysis. The process has been carried out in the following conditions: pH from 0.5 to 0.1; electrolyte - copper sulphate of semi-conductor purity; metal cathode, anode - copper of 99.99% purity, temperature from 15°C to 30°C; cathodic pulse time from 10 ms to 50 ms; current switch-off time from 1 to 3s; cathodic current density from 40 to 100 mA/cm². The solution has been mixed using a magnetic stirrer and consisted of the following additions: animal glue from 0.02 ml/1 to 0:2 ml/1 and NaCl from 0.2 ml/1 to 1 ml/1.

An example of the production of copper nanoparticles in ionic liquids, which are not aqueous solutions, is described in YU et al: "Electro-reduction of cuprous chloride powder to copper nanoparticles in an ionic liquid", ELECTROCHEMISTRY COMMUNICATION, vol. 9, no. 6, 1 June 2007, pages 1374-1381.

It appears from the above mentioned prior art electrochemical methods for obtaining copper nanopowders that they require costly preparation of substrate (solutions, reagents of appropriate purity, reduction reagents and other reagents). These processes are so complicated and expensive that the nanopowders market prices are very high.

One of the fundamental conditions ensuring technological feasibility and economic viability of metal recovery from industrial electrolytes of low concentration of deposited elements is providing sufficient mass transport rates to the electrode of electrodeposited ions. This way the rate and efficiency of nanopowder production process is increased.

The present invention solves the problem of the necessity of using an electrolyte of appropriate purity and concentration, and of using additional electrolytes and other substances. It has been unexpectedly found out that the copper powders and nanopowders can be obtained from industrial electrolyte solutions including the waste waters if they undergo potentiostatic pulse electrolysis without the current direction change and with the current direction change using ultramicroelectrodes.

The method for obtaining copper powders and nanopowders from industrial electrolytes and waste waters through electrodeposition of metallic copper on a cathode according to said invention consists in that, that the electrolyte solution of copper ions concentration higher than 0.01 g dm⁻³ undergoes potentiostatic pulse electrolysis without the current direction change or with the current direction change using the cathode potential value close to the plateau or on the plateau of the current voltage curve shown in Fig. 1 on which the plateau of the current potential range is from -0.2 V ÷ -1 V, a moveable or static ultramicroelectrode or an array of ultramicroelectrodes made of gold, platinum or stainless steel wire or foil is used as a cathode, whereas metallic copper is used as an anode and the process is carried out at temperature from 18-60°C, and the electrolysis lasts from 0.005 s to 60 s.

The advantage of the method according to the invention consists in that, that the electrolyte solution undergoes potentiostatic electrolysis as shown in Figures 2 from a) to d) in which:
- Fig. 2a) shows a pulse in cathodic potential Eₖ in the range from -0.2V ÷ -1.0 V, in reference to copper electrode, in time tₖ from 0.005 s to 60 s,
- Fig. 2b) shows a pulse in cathodic potential *E*ₖ in the range from -0.2 V ÷ -1.0 V, in reference to copper electrode, in time *t*ₖ from 0.005 s to 60 s, and then a pulse in anodic potential *E*ₐ₁ in the range from 0.0 V ÷ +1.0 V, in reference to copper electrode, in time *t*ₐ₁ shorter for at least 10% than time *t*ₖ,
- Fig. 2c) shows a pulse in anodic potential *E*ₐ₀ in the range from 0.0 V ÷ +1.0 V, in reference to copper electrode, in time *t*ₐ₀ ≤ *t*ₖ, and then a pulse in cathodic potential *E*ₖ in the range from -0.2 V ÷ -1.0 V , in reference to copper electrode, in time *t*ₖ from 0.005s to 60s,
- Fig. 2d) shows a pulse in anodic potential *E*ₐ₀ in the range from 0.0 V ÷ +1.0 V, in reference to copper electrode, in time *t*ₐ₀ ≤ *t*ₖ, and then a pulse in cathodic potential *E*ₖ in the range from -0.2 V ÷ -1.0 V , in reference to copper electrode, in time *t*ₖ from 0.005 s to 60 s, and a subsequent pulse in anodic potential *E*ₐ₁ in time *t*ₐ₁ shorter for at least 10% than *t*ₖ.

Cathodic copper reduction process is controlled by ion diffusion to the electrode which in said method is achieved by using ultramicroelectrodes or an array of ultramicroelectrodes, and carrying out potentiostatic electrolysis at the cathodic potential close to the plateau or on the plateau of the current voltage curve (Fig. 1). Said electrolysis process can be studied using chronoamperometry consisting in current measurement as a function of time at constant potential applied to the electrode.

The diameter of wire ultramicroelectrodes used in said method can be from 1 to 100 µm. The ultramicroelectrode array area can measure from 1·10⁻⁶ cm² to 10000 cm². The area of ultramicroelectrode array in the shape of plates can measure from 1 cm² to 10000 cm².

When moveable electrodes are used the time they remain in the electrolyte is equal to the duration of one electrolysis cycle. When static electrodes are used the time they remain in the electrolyte is equal to the duration of one electrolysis cycle. After each cycle an electrode is removed from the solution and a new electrode is immersed in the electrolyte solution.

The electrolysis product, i.e. powders or nanopowders can be removed from an electrode surface using a jet stream of either inert gas or liquid or it can be removed from an electrode surface mechanically using a sharp-edged gathering device made of Teflon for example.

Using said electrochemical method, copper powders and nanopowders characterised by particle structure and dimension repeatability are obtained from industrial electrolyte solutions including waste industrial electrolytes and wastewaters from copper industry and electroplating plants. Copper nanopowders of 99%+ to 99.999% purity can be obtained using said method from waste industrial electrolytes and wastewaters without additional treatment. It allows to obtain nanopowders on an industrial scale at significantly reduced costs. Using said method, powders or nanopowders of different shapes, structure and dimensions are obtained depending on the size of the electrode, metal the electrode is made of, conditions in which the electrolysis is carried out and particularly the kind of electrolysis (Fig. 2 items a-d), temperature and copper concentration in the electrolyte.

Obtaining copper nanopowders and powders using said method is shown in the examples.

### Example I.

A platinum wire working ultramicroelectrode a diameter of which is 10 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining, composed of 46 g dm⁻³ Cu, 170-200 g dm⁻³ H₂SO_{4,} Ni, As, Fe (>1000 mg dm⁻³), Cd, Co, Bi, Ca, Mg, Pb, Sb (from 1 mg dm⁻³ to 1000 mg dm⁻³) and Ag, Li, Man, Pd, Rh (<1 mg dm⁻³) as well as animal glue and thiourea (<1 mg dm⁻³). The electrodes are connected to measuring device - Autolab GSTST30 potentiostat working on-line with a personal computer (PC) with GPES software by Eco Chemie with the aid of a BNC connector.
Parameters of the process have been as follows: ${E}_{a 0} = 0.6 V {t}_{a 0} = 0.1 s$ ${E}_{k} = - 0.4 V {t}_{k} = 0.1 s$

After electrochemical deposition of copper on the electrode the structure and dimensions of deposited powder have been studied using a scanning electron microscope and it has been stated that the obtained deposit is in the shape of tubes of about 250 nm length and about 50-70 nm width. On the basis of the analysis of energy dispersion spectrum (EDS) it has been stated that only lines characteristic of copper are present which shows the purity of the obtained product.

### Example II.

A platinum wire working ultramicroelectrode a diameter of which is 10 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V {t}_{k} = 0.125 s$

After electrochemical deposition of copper on the electrode the structure and dimensions of deposited powder have been studied using a scanning electron microscope and it has been stated that the obtained deposit is in the shape of tubes of about 600 nm length and about 60-120 nm width. On the basis of the analysis of energy dispersion spectrum (EDS) it has been stated that only lines characteristic of copper are present.

### Example III.

A platinum wire working ultramicroelectrode a diameter of which is 100 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V {t}_{k} = 0.1 s$

After electrochemical deposition of copper on the electrode the structure and dimensions of deposited powder have been studied using a scanning electron microscope and it has been stated that the obtained deposit is in the shape of large crystallites of about 200 nm-600 nm grain diameter. On the basis of the analysis of energy dispersion spectrum (EDS) it has been stated that only lines characteristic of copper are present.

### Example IV.

A gold wire working ultramicroelectrode a diameter of which is 10 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V {t}_{k} = 0.125 s$

After electrochemical deposition of copper on the electrode the structure and dimensions of deposited powder have been studied using a scanning electron microscope and it has been stated that the obtained deposit is in the shape of large crystallites of about 150 nm grain diameter. On the basis of the analysis of energy dispersion spectrum (EDS) it has been stated that only lines characteristic of copper are present.

### Example V.

A gold wire working ultramicroelectrode a diameter of which is 40 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V {t}_{k} = 0.5 s$

After electrochemical deposition of copper on the electrode the structure and dimensions of deposited powder have been studied using a scanning electron microscope and it has been stated that the obtained deposit is in the spherical shape of about 250- 300 nm diameter. On the basis of the analysis of energy dispersion spectrum (EDS) it has been stated that only lines characteristic of copper are present.

### Example VI.

A gold wire working ultramicroelectrode a diameter of which is 40 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s .$ ${E}_{k} = - 0.5 V {t}_{k} = 0.1 s$

After electrochemical deposition of copper on the electrode the structure and dimensions of deposited powder have been studied using a scanning electron microscope and it has been stated that the obtained deposit is in the spherical shape of about 250-300 nm diameter. On the basis of the analysis of energy dispersion spectrum (EDS) it has been stated that only lines characteristic of copper are present.

### Example VII.

A stainless steel wire working ultramicroelectrode a diameter of which is 25 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are - connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V {t}_{k} = 0.05 and t = 0.075 s$

After electrochemical deposition of copper on the electrode the structure and dimensions of deposited powder have been studied using a scanning electron microscope and it has been stated that the obtained deposit is in the spherical shape. The grain diameter is of about 300 nm for *t* = 0.05 s and about 400 nm for *t* = 0.075 s. On the basis of the analysis of energy dispersion spectrum (EDS) it has been stated that only lines characteristic of copper are present.

### Example VIII.

A stainless steel wire working ultramicroelectrode a diameter of which is 25 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.45 V {t}_{k} = 0.05 s and t = 0.075 s$

After electrochemical deposition of copper on the electrode the structure and dimensions of deposited powder have been studied using a scanning electron microscope and it has been stated that the obtained deposit is in the spherical shape. The grain diameter is of about 200 nm for *t* = 0.05 s and about 550 nm for *t* = 0.075 s. On the basis of the analysis of energy dispersion spectrum (EDS) it has been stated that only lines characteristic of copper are present.

### Example IX.

A stainless steel wire working ultramicroelectrode a diameter of which is 25 µm, serving as a cathode and a reference electrode (an anode) in the form of a copper plate, the area of which is 0.3 cm² and its thickness is 0.1 cm are immersed in industrial electrolyte as in Example I with Cu content of 46 g dm⁻³ placed in an electrochemical cell thermostated up to 25°C. The electrodes are connected to measuring device - potentiostat working on-line with a personal computer (PC) with special software.

Parameters of the process have been as follows: ${E}_{a} = 0.6 V {t}_{a 0} = 0.1 s$ ${E}_{k} = - 0.5 V {t}_{k} = 0.05 s and t = 0.075 s$

After electrochemical deposition of copper on the electrode the structure and dimensions of deposited powder have been studied using a scanning electron microscope and it has been stated that the obtained deposit is in the spherical shape. The grain diameter is of about 600-700 nm for *t* = 0.05 s and about 700-800 nm for *t* = 0.075 s. On the basis of the analysis of energy dispersion spectrum (EDS) it has been stated that only lines characteristic of copper are present.

### Example X.

A stainless steel wire working ultramicroelectrode a diameter of which is 25 µm, serving as a cathode and a reference electrode (an anode) in the form of a copper plate, the area of which is 0.3 cm² and its thickness is 0.1 cm are placed in an electrochemical cell thermostated up to 25°C. The cell is filled with industrial electrolyte, used in copper electrorefining the composition of which is given in Example I. The electrodes are connected to measuring device - potentiostat working on-line with a personal computer (PC) with special software.

Parameters of the process have been as follows: ${E}_{a 0} = 0.6 V {t}_{a 0} = 0.1 s$ ${E}_{k} = - 0.4 V and {E}_{k} = - 0.45 V {t}_{k} = 0.1 s$

After electrochemical deposition of copper on the electrode the structure and dimensions of deposited powder have been studied using a scanning electron microscope and it has been stated that the obtained deposit is in the spherical shape of distinct structure. The grain diameter is in the range from 200-1200 nm. On the basis of the analysis of energy dispersion spectrum (EDS) it has been stated that only lines characteristic of copper are present.

### Example XI.

A cathode - a stainless steel plate of an area of about 1 cm² and an anode in the form of a copper plate of an area of 3 cm² and thickness of 0.1 cm are immersed in industrial electrolyte the composition of which is given in Example I. The electrodes are connected to measuring device - potentiostat working on-line with a personal computer (PC) with special software.

Parameters of the process have been as follows: ${E}_{k} = - 0.4 V {t}_{k} = 1 s , {t}_{k} = 15 s , {t}_{k} = 30 s , {t}_{k} = 60 s .$

After electrochemical deposition of copper on the electrode the structure and dimensions of deposited powder have been studied using a scanning electron microscope and it has been stated that the obtained deposit is in the spherical shape of distinct structure. The sizes of obtained agglomerates are respectively: about 5-10 µm, 2.5-3 µm, 1-2 µm, 0.2-0.5 µm for the following times 60, 30, 15, 1s respectively. On the basis of the analysis of energy dispersion spectrum (EDS) it has been stated that only lines characteristic of copper are present.

### Example XII.

A stainless steel wire working ultramicroelectrode a diameter of which is 25 µm, serving as a cathode and a reference electrode (an anode) in the form of a copper plate, the area of which is 0.3 cm² and its thickness is 0.1 cm are placed in an electrochemical cell thermostated up to 25°C. The cell is filled with spent industrial electrolyte, used in copper electrorefining composed of 0.189 g dm⁻³ Cu, 170-200 g dm⁻³ H₂SO₄, Ni, As, Fe (>1000 mg dm⁻³), Cd, Co, Bi, Ca, Mg, Pb, Sb (from 1 mg dm⁻³ to 1000 mg dm⁻³ and Ag, Li, Mn, Pd, Rh (<1 mg dm⁻³) as well as animal glue and thiourea. The electrodes are connected to measuring device - potentiostat working on-line with a personal computer (PC) with special software.

Parameters of the process have been as follows: ${E}_{k} = - 0.4 V {t}_{k} = 0.5 s$

After electrochemical deposition of copper on the electrode the structure and dimensions of deposited powder have been studied using a scanning electron microscope and it has been stated that the obtained deposit is in the spherical shape of distinct structure. The grain diameter is in the range from 350 nm to 2.5 µm. On the basis of the analysis of energy dispersion spectrum (EDS) it has been stated that only lines characteristic of copper are present.

## Claims

1. The method for obtaining copper powders and nanopowders from industrial waste water electrolytes through electrochemical deposition of copper on a cathode, wherein the electrolyte solution of copper ion concentration higher than 0.01 gdm⁻³ undergoes potentiostatic pulse electrolysis, using the cathode potential range of from -0.2V to -1V, in reference to copper electrode; a cathode ultramicroelectrode, the ultramicroelectrode comprising gold, platinum or stainless steel, or an array of ultramicroelectrodes, the ultramicroelectrodes comprising gold, platinum or stainless steel; an anode comprising metallic copper, the process being carried out at temperature of from 18-60°C, and the electrolysis lasting for a period of 0.005 to 60s.

2. The method according to claim 1, **characterised in that** the electrolyte solution undergoes potentiostatic electrolysis according to one or more of the processes which:
- a) show a pulse in cathodic potential Eₖ in the range from -0.2V to -1.0V, in reference to copper electrode, in time tₖ from 0.005s to 60s,
- b) show a pulse in cathodic potential Eₖ in the range from -0.2V to -1.0V, in reference to copper electrode, in time tₖ from 0.005s to 60s, and then a pulse in anodic potential Eₐ₁ in the range from 0.0V to +1.0V, in reference to copper electrode, in time tₐ₁ shorter for at least 10% than time tₖ,
- c) show a pulse in anodic potential Eₐ₀ in the range from 0.0V to +1.0V, in reference to copper electrode, in time tₐ₀ ≤ tₖ, and then a pulse in cathodic potential Eₖ in the range from -0.2V to -1.0V , in reference to copper electrode, in time tₖ from 0.005s to 60s,
- d) show a pulse in anodic potential Eₐ₀ in the range from 0.0V to +1.0V, in reference to copper electrode, in time tₐ₀ ≤ tₖ and then a pulse in cathodic potential Eₖ in the range from -0.2V to -1.0V, in reference to copper electrode, in time tₖ from 0.005s to 60s, and a subsequent pulse in anodic potential Eₐ₁ in time tₐ₁ shorter for at least 10% than tₖ.

3. A method according to claim 1, wherein the potentiostatic pulse electrolysis takes place with a change in current direction.

4. A method according to claim 1, wherein the potentiostatic pulse electrolysis takes place without a change in current direction.

5. A method according to claim 1, wherein the ultramicroelectrode is a moveable ultramicroelectrode.

6. A method according to claim 1, wherein the ultramicroelectrode is a static ultramicroelectrode.

7. A method according to claim 1, wherein the ultramicroelectrode has an array area of from 1 x 10⁻⁶ to 10000 cm².

8. A method according to claim 3 wherein the anodic potential Eₐ₀ is 0.6V.

9. A method according to claim 9 wherein the cathodic potential Eₖ is 0.4V, -0.45V or -0.5V.

10. A method according to claim 9 wherein the pulse in the anodic potential is for a period (tₐ₀) of 0.1s.

11. A method according to claim 10 wherein the cathodic potential Eₖ is 0.4V, and the pulse in the cathodic potential is for a period (tₖ) of about 0.1 s.

12. A method according to claim 1 wherein the ultramicroelectrode has a diameter of from 1-100µm,

13. An apparatus for obtaining copper powders and nanopowders from electrolytes through electrochemical deposition of copper on a cathode, comprising an electrolyte having a copper ion concentration higher than 0.01 gdm⁻³; means for providing a potentiostatic pulse electrolysis; a cathode comprising gold, platinum or stainless steel, or an array of electrodes, the electrodes comprising gold, platinum or stainless steel; an anode comprising metallic copper; and means for providing a process temperature of from 18-60°C, and means for maintaining the electrolysis from 0.005 to 60s
**characterised in that** the cathode is an ultramicroelectrode or that the array of electrodes is an array of ultramicroelectrodes;
and further **characterised in that** the electrolytes are industrial waste water electrolytes.

## Patentansprüche

1. Verfahren für die Gewinnung von Kupferpulvern und -nanopulvern aus Elektrolyten von industriellem Abwasser durch elektrochemische Abscheidung von Kupfer auf einer Kathode, wobei die Elektrolytlösung der Kupferionenkonzentration von höher als 0,01 gdm⁻³ eine potentiostatische Pulselektrolyse durchläuft, unter Verwendung des Kathodenpotenzialbereichs von -0,2 V bis -1 V in Bezug auf die Kupferelektrode; einer kathodischen Ultramikroelektrode, wobei die Ultramikroelektrode Gold, Platin oder Edelstahl umfasst, oder eines Arrays von Ultramikroelektroden, wobei die Ultramikroelektroden Gold, Platin oder Edelstahl umfassen; einer Anode, die metallisches Kupfer umfasst, wobei der Prozess bei einer Temperatur von 18-60 °C durchgeführt wird und die Elektrolyse für einen Zeitraum von 0,005 bis 60 s dauert.

2. Verfahren nach Anspruch 1, **dadurch gekennzeichnet, dass** die Elektrolytlösung eine potentiostatische Elektrolyse nach einem oder mehreren der Prozesse durchläuft, die
- a) einen Puls im kathodischen Potenzial Eₖ im Bereich von -0,2 V bis -1,0 V, in Bezug auf die Kupferelektrode, in der Zeit tₖ von 0,005 s bis 60 s zeigen,
- b) einen Puls im kathodischen Potenzial Eₖ im Bereich von -0,2 V bis -1,0 V, in Bezug auf die Kupferelektrode, in der Zeit tₖ von 0,005 s bis 60 s und dann einen Puls im anodischen Potenzial Eₐ₁ im Bereich von 0,0 V bis +1,0 V, in Bezug auf die Kupferelektrode, in der Zeit tₐ₁, die mindestens 10 % kürzer als Zeit tₖ ist, zeigen,
- c) einen Puls im anodischen Potenzial Eₐ₀ im Bereich von 0,0 V bis +1,0 V, in Bezug auf die Kupferelektrode, in der Zeit tₐ₀ ≤ tₖ und dann einen Puls im kathodischen Potenzial Eₖ im Bereich von -0,2 V bis -1,0 V, in Bezug auf die Kupferelektrode, in der Zeit tₖ von 0,005 s bis 60 s zeigen,
- d) einen Puls im anodischen Potenzial Eₐ₀ im Bereich von 0,0 V bis +1,0 V, in Bezug auf die Kupferelektrode, in der Zeit tₐ₀ ≤ tₖ und dann einen Puls im kathodischen Potenzial Eₖ im Bereich von -0,2 V bis -1,0 V, in Bezug auf die Kupferelektrode, in der Zeit tₖ von 0,005 s bis 60 s und einen anschließenden Puls im anodischen Potenzial Eₐ₁ in der Zeit tₐ₁, die mindestens 10 % kürzer als Zeit tₖ ist, zeigen.

3. Verfahren nach Anspruch 1, wobei die potentiostatische Pulselektrolyse mit einer Veränderung der Stromrichtung stattfindet.

4. Verfahren nach Anspruch 1, wobei die potentiostatische Pulselektrolyse ohne eine Veränderung der Stromrichtung stattfindet.

5. Verfahren nach Anspruch 1, wobei die Ultramikroelektrode eine bewegliche Ultramikroelektrode ist.

6. Verfahren nach Anspruch 1, wobei die Ultramikroelektrode eine statische Ultramikroelektrode ist.

7. Verfahren nach Anspruch 1, wobei die Ultramikroelektrode eine Array-Fläche von 1 x 10⁻⁶ bis 10000 cm² aufweist.

8. Verfahren nach Anspruch 3, wobei das anodische Potenzial Eₐ₀ 0,6 V beträgt.

9. Verfahren nach Anspruch 9, wobei das kathodische Potenzial Eₖ 0,4 V, -0,45 V oder -0,5 V beträgt.

10. Verfahren nach Anspruch 9, wobei der Puls in dem anodischen Potenzial für einen Zeitraum (tₐ₀) von 0,1 s erfolgt.

11. Verfahren nach Anspruch 10, wobei das kathodische Potenzial Eₖ 0,4 V beträgt und der Puls in dem kathodischen Potenzial für einen Zeitraum (tₖ) von etwa 0,1 s s erfolgt.

12. Verfahren nach Anspruch 1, wobei die Ultramikroelektrode einen Durchmesser von 1-100 µm aufweist.

13. Vorrichtung für die Gewinnung von Kupferpulvern und -nanopulvern aus Elektrolyten durch elektrochemische Abscheidung von Kupfer auf einer Kathode, die Folgendes umfasst: einen Elektrolyten, der eine Kupferionenkonzentration von höher als 0,01 gdm⁻³ aufweist; Mittel für die Bereitstellung einer potentiostatischen Pulselektrolyse; eine Kathode, die Gold, Platin oder Edelstahl umfasst, oder ein Array von Elektroden, wobei die Elektroden Gold, Platin oder Edelstahl umfassen; eine Anode, die metallisches Kupfer umfasst; und Mittel für die Bereitstellung einer Prozesstemperatur von 18-60 °C und Mittel für die Aufrechterhaltung der Elektrolyse von 0,005 bis 60 s,
**dadurch gekennzeichnet, dass** die Kathode eine Ultramikroelektrode ist oder dass der Array von Elektroden ein Array von Ultramikroelektroden ist;
und weiter **dadurch gekennzeichnet, dass** die Elektrolyten Elektrolyten von industriellem Abwasser sind.

## Revendications

1. Procédé permettant d'obtenir des poudres et des nanopoudres de cuivre à partir d'électrolytes d'eaux usées industrielles par dépôt électrochimique du cuivre sur une cathode, où une solution d'électrolytes ayant une concentration en ions cuivre supérieure à 0,01 g/dm⁻³ est soumise à une électrolyse potentiostatique en régime pulsé en utilisant une plage de potentiels cathodiques qui va de -0,2 V à -1 V par rapport à une électrode au cuivre ; une ultramicroélectrode cathodique, l'ultramicroélectrode étant à base d'or, de platine ou d'acier inoxydable, ou un réseau d'ultramicroélectrodes, les ultramicroélectrodes étant à base d'or, de platine ou d'acier inoxydable ; une anode à base de cuivre métallique ; le procédé étant effectué à une température de 18-60 °C et la durée de l'électrolyse allant de 0,005 à 60 s.

2. Procédé selon la revendication 1, **caractérisé en ce que** la solution d'électrolytes est soumise à une électrolyse potentiostatique effectuée conformément à un ou plusieurs des protocoles suivants :
- a) protocole utilisant une impulsion à un potentiel cathodique Eₖ dans la plage de -0,2 V à -1,0 V par rapport à une électrode au cuivre sur une période d'une durée tₖ qui va de 0,005 s à 60 s,
- b) protocole utilisant une impulsion à un potentiel cathodique Eₖ dans la plage de -0,2 V à -1,0 V par rapport à une électrode au cuivre sur une période d'une durée tₖ qui va de 0,005 s à 60 s puis une impulsion à un potentiel anodique Eₐ₁ dans la plage de 0,0 V à +1,0 V par rapport à une électrode au cuivre sur une période d'une durée tₐ₁ qui est au moins 10 % plus courte que la période tₖ,
- c) protocole utilisant une impulsion à un potentiel anodique Eₐ₀ dans la plage de 0,0 V à +1,0 V par rapport à une électrode au cuivre sur une période d'une durée tₐ₀ ≤ tₖ puis une impulsion à un potentiel cathodique Eₖ dans la plage de -0,2 V à -1,0 V par rapport à une électrode au cuivre sur une période d'une durée tₖ qui va de 0,005 s à 60 s,
- d) protocole utilisant une impulsion à un potentiel anodique Eₐ₀ dans la plage de 0,0 V à +1,0 V par rapport à une électrode au cuivre sur une période d'une durée tₐ₀ ≤ tₖ puis une impulsion à un potentiel cathodique Eₖ dans la plage de -0,2 V à -1,0 V par rapport à une électrode au cuivre sur une période d'une durée tₖ qui va de 0,005 s à 60 s suivie d'une impulsion à un potentiel anodique Eₐ₁ sur une période d'une durée tₐ₁ qui est au moins 10 % plus courte que tₖ.

3. Procédé selon la revendication 1, où l'électrolyse potentiostatique en régime pulsé est effectuée avec une modification de la direction du courant.

4. Procédé selon la revendication 1, où l'électrolyse potentiostatique en régime pulsé est effectuée sans modification de la direction du courant.

5. Procédé selon la revendication 1, où l'ultramicroélectrode est une ultramicroélectrode mobile.

6. Procédé selon la revendication 1, où l'ultramicroélectrode est une ultramicroélectrode statique.

7. Procédé selon la revendication 1, où la zone de réseau de l'ultramicroélectrode va de 1 x 10⁻⁶ à 10 000 cm².

8. Procédé selon la revendication 3, où le potentiel anodique Eₐ₀ est de 0,6 V.

9. Procédé selon la revendication 9, où le potentiel cathodique Eₖ est de -0,4 V, -0,45 V ou -0,5 V.

10. Procédé selon la revendication 9, où la durée de l'impulsion au potentiel anodique (tₐ₀) est de 0,1 s.

11. Procédé selon la revendication 10, où le potentiel cathodique Eₖ est de -0,4 V et où la durée de l'impulsion au potentiel cathodique (tₖ) est de 0,1 s environ.

12. Procédé selon la revendication 1, où le diamètre de l'ultramicroélectrode est de 1-100 µm.

13. Appareil permettant d'obtenir des poudres et des nanopoudres de cuivre à partir d'électrolytes par dépôt électrochimique du cuivre sur une cathode, comprenant un électrolyte ayant une concentration en ions cuivre supérieure à 0,01 g/dm⁻³ ; un moyen permettant d'effectuer une électrolyse potentiostatique en régime pulsé ; une cathode à base d'or, de platine ou d'acier inoxydable ou un réseau d'électrodes, les électrodes étant à base d'or, de platine ou d'acier inoxydable ; une anode à base de cuivre métallique ; et des moyens permettant de maintenir une température de 18-60 °C pendant le procédé et de poursuivre l'électrolyse pendant 0,005 à 60 s,
**caractérisé en ce que** la cathode est une ultramicroélectrode ou **en ce que** le réseau d'électrodes est un réseau d'ultramicroélectrodes ;
et en outre **caractérisé en ce que** les électrolytes sont des électrolytes d'eaux usées industrielles.
